

Nov. 29, 1955

D. R. MOREY

2,725,297

ANTISTATIC PHOTOGRAPHIC FILM

Filed Oct. 8, 1952



DONALD R. MOREY  
INVENTOR.

BY *Daniel J. Mayne*  
*R. Frank Smith*  
ATTORNEYS

## 1

2,725,297

## ANTISTATIC PHOTOGRAPHIC FILM

Donald R. Morey, Rochester, N. Y., assignor to Eastman Kodak Company, Rochester, N. Y., a corporation of New Jersey

Application October 8, 1952, Serial No. 313,771

6 Claims. (Cl. 95—9)

This invention relates to photographic film and particularly to a film protected against static.

The accumulation of electrical charges on photographic film has been the cause of considerable trouble. These charges are produced by the friction of the film moving over rollers or past the gates of a camera, or by the separation of the emulsion from the backing side, upon unreeing of a large roll, and when discharged are manifested as irregular fogged patterns in the emulsion of the film after it has been developed. These static effects are particularly noticeable in films provided with cellulose nitrate supports, although they are also evident on cellulose acetate supports, particularly since the advent of high speed emulsions. Static markings on film are thought to result also upon separation of emulsion from paper during unwinding of a stock roll when the roll was wound at a humidity sufficiently high to impart sticking.

Attempts have been made to overcome static in photographic film by the application of various layers to the film support. These layers have in general consisted of materials designed to dissipate the electric charges by providing the film with a conducting surface. Materials which absorb moisture and therefore provide a conducting surface have frequently been employed. Most of these methods have not proven entirely satisfactory with the newer high speed emulsions.

It is also known that antistatic layers may be made by adding to gelatin certain ionic organic materials including water-soluble polymeric materials as described in Morey and White U. S. Patent 2,639,234. The use of water-soluble inorganic acid salts in antistatic layers has also been proposed. None of these types of antistatic coating has, however, been broadly satisfactory for all of the different film types which are manufactured.

It is therefore an object of the present invention to provide a novel and effective means of protecting a sensitive photographic film against static. A further object is to provide a method of coating a photographic film in order to reduce its static tendency. A still further object is to provide a suitable means for protecting cellulose acetate films especially cellulose triacetate films against static. A further object is to provide means of producing photographic film of considerably lower electrical resistance while, at the same time, retaining its optical transparency. Other objects will appear from the following description of my invention.

These objects are accomplished by coating photographic film base with a mixture of three components: (1) gelatin, (2) a water-soluble polymeric salt, and (3) a water-soluble simple inorganic acid salt.

The accompanying drawing shows a sectional view of film constructed according to my invention.

The ternary mixture of gelatin, water-soluble polymeric salt, and water-soluble simple inorganic acid salt which I propose to use produces an enhanced conductivity over that of the sum of the separate components. There is

## 2

a marked synergistic effect of the mixture which enables the desired conductance level to be reached without having to have excessive amounts of addenda which would otherwise lead to incompatibility and a hazy or sticky coating.

It has been found possible to add sufficient of these addenda to bring the surface resistivity below  $10^{10}$  ohms, a value which is sufficient to alleviate difficulties from static electricity generated in the normal handling of the film. The surface resistance of the usual gelatin backing is 50 to 100 times the value stated above.

The surface resistivity was measured placing two parallel electrodes on the film at a fixed relative humidity of 50%; these electrodes are long compared to the distance between them, so as to avoid end effects. The observed resistance reading is divided by the distance between electrodes and multiplied by their length, to obtain the surface resistivity.

The ternary mixtures which I propose to use contain the following ingredients:

1. Gelatin.
2. Water-soluble polymeric salt, e. g.;  
Carboxy methyl cellulose (sodium salt).  
Sodium alginate.  
25 Sodium cellulose sulfate.  
Cellulose acetate sodium sulfate.  
Methyl methacrylate-methacrylic acid (sodium salt).  
Sulfonated polystyrene (sodium salt).  
Sodium polyethylene glycol lauroyl sulfate.
- 30 3. Water-soluble, simple inorganic acid salt, e. g. sodium chloride.

When used to prevent static on sensitive photographic film the mixtures of my invention may be incorporated in the sensitive emulsion layer in an overcoating layer or used as a backing layer. Our agents possess such physical properties that when applied to the back of a cellulose ester film they form a clear transparent layer on the film without any undesirable physical or photographic effects.

40 It is, of course, assumed that the addenda will be properly chosen or purified so that they have no fogging or desensitizing action upon light-sensitive emulsions. Our ternary mixtures are preferably applied to the back of the film, that is, to the side opposite that of the sensitive emulsion layer.

The following examples illustrate methods of applying the ternary mixture to films according to my invention.

## Example 1

50 To an aqueous gelatin solution containing 5% of gelatin there was added 20% of the weight of the gelatin of the sodium salt of carboxymethyl cellulose and 2% of the weight of the gelatin of sodium chloride. This solution was applied as a backing to a roll of subbed cellulose triacetate film base by means of a dip roller and dried. The film was then further coated on the reverse side with a suitable subbing layer and a gelatin-silver halide emulsion. This film showed good optical appearance of the backing. Films similarly coated with gelatin alone and with gelatin plus 20% of the weight of the gelatin of the sodium salt of carboxymethyl cellulose and with gelatin plus 2% of the weight of gelatin of sodium chloride were brought to equilibrium with 50% relative humidity and tested for electrical conductance. (In computing the sum of the separate conductances, the value for the gelatin check coating was subtracted, since gelatin would otherwise be added twice, i. e. with the sodium chloride and with the polymer salt.) The following results for electrical conductance were obtained (in the

tables, the value for "ohms" is the reciprocal ohms reading):

|                                                       | $1/R \times 10^{10}$ ohms |
|-------------------------------------------------------|---------------------------|
| Gelatin check coating                                 | 0.069                     |
| Gelatin+20 percent Na salt of carboxymethyl cellulose | 3.23                      |
| Gelatin+2 percent NaCl                                | 0.38                      |
| Sum of separate conductances of the components        | 3.54                      |
| Gelatin+20 percent CMC+2 percent NaCl                 | 8.33                      |

A synergistic factor of over 2 was obtained.

Similar tests were made using other polymer salts with the following results.

*Example 2*

|                                                | Ohms  |
|------------------------------------------------|-------|
| Gelatin check coating                          | 0.011 |
| Gelatin+20 percent sodium alginate             | 1.47  |
| Gelatin+2 percent NaCl                         | 0.141 |
| Sum of separate conductances of the components | 1.60  |
| Gelatin+20 percent Na alginate+2 percent NaCl  | 6.25  |

A synergistic factor of nearly 4 was obtained.

*Example 3*

|                                                            | Ohms  |
|------------------------------------------------------------|-------|
| Gelatin check coating                                      | 0.014 |
| Gelatin+10 percent sodium cellulose sulfate                | 0.045 |
| Gelatin+2 percent NaCl                                     | 0.068 |
| Sum of separate conductances of the components             | 0.099 |
| Gelatin+10 percent sodium cellulose sulfate+2 percent NaCl | 0.217 |

A synergistic factor of 2 was obtained.

*Example 4*

|                                                            | Ohms  |
|------------------------------------------------------------|-------|
| Gelatin check coating                                      | 0.014 |
| Gelatin+20 percent sodium cellulose sulfate                | 0.061 |
| Gelatin+2 percent NaCl                                     | 0.068 |
| Sum of separate conductances of the components             | 0.115 |
| Gelatin+20 percent sodium cellulose sulfate+2 percent NaCl | 0.333 |

A synergistic factor of 3 was obtained.

*Example 5*

|                                                                                  | Ohms |
|----------------------------------------------------------------------------------|------|
| Gelatin check coating                                                            | 0.06 |
| Gelatin+20 percent copolymer of methyl methacrylate-methacrylic acid sodium salt | 2.12 |
| Gelatin+2 percent NaCl                                                           | 0.35 |
| Sum of separate conductances of the components                                   | 2.41 |
| Gelatin+20 percent copolymer plus 2 percent NaCl                                 | 18.5 |

A synergistic factor of 8 was obtained.

*Example 6*

|                                                | Ohms |
|------------------------------------------------|------|
| Gelatin check coating                          | 0.06 |
| Gelatin+20 percent copolymer                   | 2.12 |
| Gelatin+4 percent NaCl                         | 2.78 |
| Sum of separate conductances of the components | 4.84 |
| Gelatin+20 percent copolymer+4 percent NaCl    | 125. |

A synergistic factor of 26 was obtained.

*Example 7*

|                                                          | Ohms |
|----------------------------------------------------------|------|
| Gelatin check coating                                    | 0.01 |
| Gelatin+20 percent Na salt of sulfonated polystyrene     | 0.18 |
| Gelatin+2 percent NaCl                                   | 0.1  |
| Sum of separate conductances of the components           | 0.27 |
| Gelatin+20 percent sulfonated polystyrene+2 percent NaCl | 1.1  |

A synergistic factor of 4 was obtained.

In my coatings as finally dried, the gelatin should comprise at least 75% by weight of the ternary mixture;

the water-soluble polymeric salt should comprise between about 5 and 20% or slightly more, of the weight of the gelatin and the simple inorganic acid salt should comprise from about 2 to 10% or slightly more, of the weight of the gelatin.

In the accompanying drawing,

The single figure is a sectional view of a film constructed according to my invention. As shown therein, a suitably subbed film support 10 of any appropriate film base material such as cellulose acetate has coated thereon a gelatin-silver halide emulsion 11 and on the opposite side a layer 12 of gelatin, water-soluble polymeric salt and water-soluble simple inorganic acid salt.

It will be understood that my invention is capable of numerous modifications within the scope of the appended claims.

I claim:

1. An antistatic photographic film comprising a cellulose ester support having thereon a sensitive silver halide emulsion layer and in one of the layers of the film a mixture of (1) gelatin, (2) a water-soluble polymeric salt selected from the group consisting of water-soluble salts of carboxymethyl cellulose, alginic acid, cellulose acid sulfate, cellulose acetate acid sulfate, methyl methacrylate-methacrylic acid, sulfonated polystyrene and polyethylene glycol lauroyl acid sulfate, and (3) from about 2% to 10% of the weight of gelatin of sodium chloride, said gelatin comprising at least 75% by weight of said mixture.

2. An antistatic photographic film comprising a cellulose ester support having one one side thereon a sensitive silver halide emulsion layer, and on the opposite side thereof a layer comprising a mixture of gelatin, the sodium salt of carboxymethyl cellulose, and from about 2% to 10% of the weight of gelatin of sodium chloride, said gelatin comprising at least 75% of said mixture.

3. An antistatic photographic film comprising a cellulose ester support having on one side thereon a sensitive silver halide emulsion layer, and on the opposite side thereof a layer comprising a mixture of gelatin, sodium alginate, and from about 2% to 10% of the weight of gelatin of sodium chloride, said gelatin comprising at least 75% of said mixture.

4. An antistatic photographic film comprising a cellulose ester support having on one side thereon a sensitive silver halide emulsion layer, and on the opposite side thereof a layer comprising a mixture of gelatin, sodium cellulose sulfate, and from about 2% to 10% of the weight of gelatin of sodium chloride, said gelatin comprising at least 75% of said mixture.

5. An antistatic photographic film comprising a cellulose ester support having on one side thereon a sensitive silver halide emulsion layer, and on the opposite side thereof a layer comprising a mixture of gelatin, cellulose acetate sodium sulfate, and from about 2% to 10% of the weight of gelatin of sodium chloride, said gelatin comprising at least 75% of said mixture.

6. An antistatic photographic film comprising a cellulose ester support having on one side thereon a sensitive silver halide emulsion layer, and on the opposite side thereof a layer comprising a mixture of gelatin, the sodium salt of methyl-methacrylate-methacrylic acid, and from about 2% to 10% of the weight of gelatin of sodium chloride, said gelatin comprising at least 75% of said mixture.

**References Cited in the file of this patent**

**UNITED STATES PATENTS**

- |    |           |                 |               |
|----|-----------|-----------------|---------------|
| 70 | 1,981,102 | Hagedorn et al. | Nov. 20, 1934 |
|    | 2,118,059 | Slack et al.    | May 24, 1938  |
|    | 2,127,621 | Staud et al.    | Aug. 23, 1938 |
|    | 2,322,085 | Yutzy           | June 15, 1943 |
|    | 2,357,590 | Jaffe           | Sept. 5, 1944 |
| 75 | 2,386,167 | Murray          | Oct. 2, 1945  |